

## UNITED STATES PATENT OFFICE.

CHRISTIAN BERGH BACKER, OF BERGEN, NORWAY.

## METHOD OF PRODUCING A PROTECTIVE COATING ON OBJECTS OF MAGNESIUM OR MAGNESIUM ALLOYS.

No Drawing.

Application filed December 16, 1921. Serial No. 522,941.

REISSUED

*To all whom it may concern:*

Be it known that I, CHRISTIAN BERGH BACKER, a subject of the King of Norway, residing at Bergen, Norway, have invented 5 certain new and useful Improvements in Methods of Producing a Protective Coating on Objects of Magnesium or Magnesium Alloys; and I do hereby declare the following to be a full, clear, and exact description 10 of the invention, such as will enable others skilled in the art to which it appertains to make and use the same.

This invention has for its object a method 15 of treating objects or materials of magnesium or magnesium alloys so as to produce upon the metal a strongly adhering coating of substantial thickness.

According to the invention such coatings are produced from the metal itself by sub- 20 jecting it to an oxidizing treatment, the intensity and duration of which is adapted to the thickness of the coating to be produced.

The coating is suitably produced by sub- 25 jecting the objects or materials, which may consist of magnesium or a magnesium alloy or which may only have a surface layer of such metal or alloy—to the action of water or water vapour at a temperature above 100° C. This treatment may be carried into 30 effect under ordinary or raised pressures.

By such a treatment it is possible to obtain a compact strongly adhering coating of magnesium hydroxide, the thickness of which may be controlled by suitable variations in 35 the temperatures employed and in the duration of the treatment.

As an example may be mentioned that by heating an object of magnesium in an auto-clave under a steam-pressure of about 10 atmospheres in 15 minutes a coating of about 40 1.5 mm. thickness has been obtained and by boiling in about one hour under a pressure of about 5 atmospheres a coating of about 0.2 mm. thickness has been produced.

The coating is an electrical insulator and 45 possesses great resistance against the action of the constituents of the atmosphere. The present process is therefore adaptable to the insulation of electrical conductors, insula- 50 tors and other objects and materials for electrical use. The windings of transformers, motors, heating apparatus, etc., may with

advantage be subjected to the described treatment in the finished apparatus or the conductors may first be provided with a thin 55 layer of the coating, whereupon they may be wound in place and finally provided with a coating of the desired thickness. Insulators may be produced from magnesium alloys or magnesium by stamping or by 60 other methods, whereupon they may be subjected to the described treatment.

The coating produced in the described manner resists the influence of chemically acting substances, for example salt solutions 65 and the like and magnesium or magnesium alloys provided with the same coating may therefore be employed where such substances are present, for example in sea water (for example for crank cases and the like for ship 70 motors).

It is known to effect the insulation of aluminium conductors by providing the same with a coating of aluminium hydroxide. As compared with such aluminium hydroxide 75 coatings, the coating of magnesium hydroxide produced according to the present invention is fundamentally different in several respects for example therein that the coating may be produced in any desired 80 thickness, so that it is applicable also for high tension currents.

The coating is hard and tough and of great cohesive power and it is strongly adhering so that it does not fall off when the 85 objects are subjected to mechanical strain. By means of impregnation for example with water glass solutions during or after the process of producing same, the strength of the coating may be increased and its character 90 may be altered. When impregnation with water glass is made use of a subsequent treatment with an acid will be suitable.

The described method may also be employed for the production of objects which 95 all through consist of magnesium hydroxide, the oxidizing treatment of the shaped object being in this case continued until the entire metal is converted. In this case the objects may beforehand have been shaped of massive 100 metal or for example of a powder of the metal or alloy.

As is well known magnesium metal when boiled in water under ordinary pressure be-

comes covered with a layer of magnesium hydroxide. This layer is, however, so thin that it is unmeasurable with a micrometer, and no method was known, whereby a layer of a thickness above 0.01 mm. could be produced.

I claim:

1. Method of producing a coating upon objects and materials of magnesium and magnesium alloys which comprises heating 10 of the objects in the presence of water at a temperature of above 100° C.

2. Method of treating objects and materials of magnesium or magnesium alloys 15 which comprises heating the objects under a superatmospherical pressure at a temperature above 100° C. in the presence of water and continuing this treatment until the magnesium metal of the object has been converted into an oxygenous magnesium compound to a depth of at least 0.01 mm.

3. Method of treating materials and objects of magnesium or magnesium alloys to 25 produce an electrically insulating coating thereupon which comprises heating of the

objects under a pressure of several atmospheres at a temperature above 100° C. in the presence of water.

4. Method of producing an electrically insulating coating upon the windings of transformers, motors, and other electrical apparatus according to claim 1 which comprises producing a thin layer upon the conductors before winding, then bringing the conductors into position and then subjecting the 30 35 formed object to the oxidizing treatment until a coating of desired thickness has been produced.

5. Objects and materials of magnesium or magnesium alloys having a hard adhering coating of a thickness of at least 0.01 mm. comprising an oxygenous magnesium compound, produced from the metal itself.

In testimony that I claim the foregoing as my invention, I have signed my name in 45 presence of two subscribing witnesses.

CHRISTIAN BERGH BACKER.

Witnesses:

JOHN KRAMME,  
S. A. ANFINDSEN.